

Sept. 21, 1937.

A. T. COLWELL

2,093,771

METHOD OF MAKING COPPER COOLED VALVES

Filed Feb. 27, 1931



INVENTOR  
Archie T. Colwell

Charles Colwell ATHS.

## UNITED STATES PATENT OFFICE

2,093,771

## METHOD OF MAKING COPPER COOLED VALVES

Archie T. Colwell, Cleveland, Ohio, assignor to  
Thompson Products, Incorporated, Cleveland,  
Ohio, a corporation of Ohio

Application February 27, 1931, Serial No. 518,666

9 Claims. (Cl. 29—156.7)

This invention relates to a method of making poppet valves for internal combustion engines and particularly to extruded valves having a cooling medium therein.

The temperatures attained in the combustion chambers of automotive engines closely approximate the temperatures to which the metals used in the manufacture of valves are heated in such manufacture. The gases which pass the exhaust valves maintain the exhaust passageway at a temperature of around 1600° F. for ordinary engine speed. These gases have a very destructive effect on the valves, causing corrosion and warping and producing a destructive change in the metal of the valve. Since these gases are directed against a portion of the valve which includes the upper portion of its stem and the lower portion of the head, it has been a problem for valve manufacturers to devise a means of cooling this portion of the valve.

This cooling has been accomplished in several ways such as providing a shield about this portion and also by filling the stem of the valve with a cooling medium which will draw the heat to a portion of the valve which may be cooled by outside means. The first of these methods is objectionable because its effect depends upon the formation of a dead air space between the protecting shield and the valve. In this type of valve the heat being directed against the protecting shield will have a destructive action on the shield and will in time eliminate the dead air space. The other method of cooling the valve, as heretofore practiced, while more permanent in nature, has been found not entirely satisfactory for the reason that it involves a considerable expense and careful planning or else the cooling medium is not very effective.

According to the present invention, a simple and inexpensive means for cooling the portion of the valve against which the exhaust gases are directed is provided.

It is an object of the present invention to produce a metallic cooled valve by a method which is inexpensive, expedient and adapted for use in large scale production of valves.

It is a further object of this invention to produce a cooled valve by a method which involves the insertion of the cooling medium in the valve blank and the forming of the valve with the insert therein.

It is a particular object of this invention to produce a metallic cooled valve by a method which includes inserting a metallic cooling medium in the valve blank and extruding the composite blank to form the valve.

This invention (in a preferred form) is illustrated in the drawing and hereinafter more fully described.

On the drawing:

Figure 1 is a sectional view of a metal blank with an insert therein and a plate welded thereto.

Figure 2 is a sectional view of a modified form of a blank.

Figure 3 is a sectional view of a further modified form of a blank.

Figure 4 is a sectional view of a valve formed by extruding the blank of Figure 2.

Figure 5 is a fragmentary sectional view of the end of a valve formed by extruding the blank of Figure 1.

Figure 6 is a sectional view of the valve showing the end of the stem in final form.

Figure 7 is a fragmentary sectional view of the end of the stem of a valve showing a modification in which the insert extends through the end of the valve.

As shown on the drawing:

In carrying out this invention, a blank 1 is formed as by casting or by cutting a slug from a bar of rolled stock. A suitable recess 2 is drilled into the blank 1. The recess is preferably cylindrical and concentric with the blank 1, extending through one end of the blank and for a substantial distance within the blank. An insert 3 is then placed in the recess 2 and forced to the inner end thereof so that when the valve is formed, in a manner hereinafter to appear, the insert will extend throughout the stem and a short distance into the head portion.

In Figure 1, the insert 3 is shown as completely filling the recess 2 and a plate 4 is welded to the end of the blank through which the recess 2 extends over the end of the insert. The purpose of the plate 4 is to prevent oxidation of the insert 3 when the blank is heated preparatory to the forming of the valve.

The blank 1 is formed of any suitable valve material, such as tungsten steel, or nickel-chromium steel. The insert 3 is made of any suitable metal such as copper which has a relatively greater rate of heat conductivity than that of the metal of the blank. The plate 4 may be made of any suitable material which will form a bond with the metal of the blank, but is preferably made of a steel having great wear resistance qualities, as this part of the blank is formed into the portion of the stem which contacts with the operating mechanism.

Figures 2 and 3 show slightly modified forms of the blank. In Figure 2, the metal plate 4 is provided with a nipple or stud 5 which fits into the recess 2 and against the insert 3. In this instance, the insert 3 is shorter than in the preceding case so as not to completely fill the recess 2. In Figure 3, a modification is shown in which instead of a metal plate there is provided a metal insert or plug 6 which is welded into the end of the recess 2 to keep the insert 3 from oxidizing during the subsequent heating of the blank.

The composite metal blank thus formed is heated to a forging temperature and extruded through a suitable die. In this operation, the blank may be extruded through a die which will 5 form the article shown in Figure 4, or in the preferred way, the metal blank is extruded so as to form a stem and a head portion thereon so as to somewhat resemble a finished valve. This intermediate blank is then finished to shape 10 by any of the known methods.

In either case the extruding process causes the formation of a head 7 and a stem 8. The insert 3 is drawn out so as to form the elongated core 9 within the stem 8. The absence of oxygen or 15 air together with the high temperature and subsequent extruding, forms a bond or welded joint between the stem 8 and core 9 which has a rate of heat conductivity closely approximating that of the metal itself whereas an ordinary joint 20 offers material resistance to the flow of heat. A portion 10 of the core 9 extends into the head 7. The metal of the plate 4 is incorporated into the end of the stem as shown at 11. This portion 11 may be finished off and provided with an 25 annular groove 12 as shown in Figure 6.

Figure 5 shows the end of the stem as it is formed when there is but a small plug 6 of metal in the blank, as shown in Figure 3.

Figure 7 shows a modified way of producing 30 the end of the stem. In this case, a length of metal at the end of the stem is removed so that the insert 9 extends through the end of the valve as shown at 13.

It will be seen that this invention, provides a 35 method of making a valve having an insert of great heat conducting properties which is economical, simple, and adapted for use in large scale production.

Many changes may be made in the design and 40 proportion of the parts and I do not wish to be limited otherwise than is necessary by the prior art and the scope of the appended claims.

I claim as my invention:

1. The method of making a cooled valve which 45 comprises forming a metal blank with a recess extending longitudinally thereof, inserting a metal having a relatively high rate of heat conductivity in said recess, welding a metal plate to said blank over the end of said recess so as to exclude air from the recess, heating the composite blank thus formed to a forging temperature and extruding the blank through a suitable die to form a head and stem thereon, the operation being carried out so that the plate 50 forms a portion of the stem and the insert is disposed longitudinally of the stem.

2. The method of making a cooled valve, which 55 comprises forming a blank of a suitable steel for making a valve, drilling a recess in said blank, placing a copper insert in said recess, welding a metal plate to said blank over the end of said recess so as to exclude oxygen from the contacting copper and steel surfaces, heating the composite metallic blank thus formed to forging 60 temperature and extruding the blank through a suitable die to form a head and stem thereon with the copper extending throughout the stem and into the head, the extruding operation being carried out so that the plate forms a portion of 65 the stem and the insert is disposed longitudinally of the stem.

3. The method of sealing a metal cooled valve, which comprises heating a valve blank having a recess therein partially filled with a metal of relatively high heat conductivity, inserting a metallic plug in the end of the recess of said blank 5 and extruding the blank to form a valve with the metal of the plug incorporated in the stem of the valve to form a part of the valve stem.

4. The method of making a cooled valve which 10 comprises forming a recess in a metal blank, placing a metallic insert in the blank, welding a metal plate to the blank over the end of the recess so as to exclude air from the recess, and extruding the blank to form a head and a stem thereon with the insert extending down the stem 15 and spread out in the head and with the plate forming a portion of the stem.

5. The method of making a cooled valve which 20 comprises forming a metal blank with a recess extending longitudinally from one end thereof into close proximity to the other end, placing a copper insert into said recess, welding a metal plug to said blank at the end of the recess so as to exclude air from the recess, heating the composite blank thus formed to a forging temperature 25 and extruding the blank through a suitable die to form a head and stem thereon with the copper spread out into the head and extending down into the stem and the plug incorporated into the blank metal to form a portion of 30 the stem.

6. The method of making a poppet valve having 35 a metal insert of high heat conductivity therein, which comprises providing a metal blank having a recess extending from one end thereof into spaced relation from the other end thereof, placing a metal having high heat conductivity characteristics in said recess and shaping the composite blank thus formed to provide a head and stem thereon with the insert metal spread 40 out into the head and extending into the stem.

7. The method of making a metal cooled valve 45 which comprises providing a metal blank having an axial blind bore therein, placing an insert metal having high heat conductivity characteristics 50 in the bore and shaping the composite blank thus formed to provide a head and stem thereon with the insert metal encased in the blank metal and spread out into the head of the valve and extending axially down the valve stem. 55

8. The method of making a copper cooled valve 60 which comprises providing a metal blank having a recess therein, filling the recess with copper and shaping the blank to provide a head and stem thereon with the copper spread out into the head to form a mushroom-shaped copper filling encased in the head and extending down the stem.

9. The method of making a metal cooled valve 65 which comprises providing a metal blank having a recess extending from one end thereof into spaced relation from the other end thereof, filling said recess with a metal having high heat conductivity characteristics and extruding the composite blank thus formed to provide a head and stem thereon with the insert metal spread out in the head to form a mushroom-shaped filling encased in the head and extending axially 70 into the stem.